

June 30, 1936.

B. GASPAR

2,046,067

METHOD OF PRODUCING COLORED PHOTOGRAPHIC MATERIALS

Filed Dec. 1, 1932

**Fig. 1.** Gelatine layer containing insoluble dyestuff salt of phenyl-amino chinolone



**Fig. 2.** Gelatine layer containing insoluble dyestuff salt



**Fig. 3.** Uncolored gelatine



**Fig. 4.** Gelatine layers containing insoluble dyestuff salts



Inventor

Bela Gaspar,

By

*D. H. Wallhauser*

Attorney

## UNITED STATES PATENT OFFICE

2,046,067

METHOD OF PRODUCING COLORED  
PHOTOGRAPHIC MATERIALS

Béla Gaspar, Brussels, Belgium

Application December 1, 1932, Serial No. 645,312  
In Germany December 2, 1931

## 3 Claims. (Cl. 95—2)

This invention relates to a method of producing colored photographic materials.

The invention may be illustrated diagrammatically by Figures 1, 2, 3 and 4 in the accompanying drawing, which shows several forms of embodiment.

In Figure 1, *c* represents the carrier or support, whilst *b* is a silver bromide gelatine layer colored, for example, with Chrysophenine G (304), which has been precipitated with hydrochloric 2-phenyl-4-aminoquinoline.

In Figure 2, *c* is the carrier or support, *b* an uncolored silver bromide gelatine layer, and *a* a gelatine layer colored, for example, with Chrysophenine G (304), which has been precipitated with hydrochloric 2-phenyl-4-aminoquinoline.

Figure 3 shows a similar material to Figure 2 with reverse order of the layers *a* and *b*, that is to say—*a* is applied to the support and *b* situated over *a*.

Figure 4 shows a form of embodiment having three differently colored silver bromide layers. *c* is a backing or support of desired material, and *d*, *e* and *f* are silver bromide gelatine layers colored as follows:—

*d* contains Diamine pure blue FF (424), *e* Chrysophenine G 304 and *f* Amidonaphthol red 6B (66). Each of these dyestuffs is precipitated in the emulsion by 2-phenyl-4-aminoquinoline.

The index numbers for the dyestuffs given in the above refer to the Schultz Dyestuff Tables, 5th Ed., 1920.

It is already known for the purpose of producing color photographs to incorporate dyestuffs in photographic layers and to fix these by a mordanting process or by the formation of a deposit. In this connection, however, it has been found that various dyestuffs reveal the tendency to separate again subsequently from the mordant. Beyond this, the inorganic salts proposed for this purpose, such as alkaline earth or heavy metal salts are very disturbing in the layer, as the same may readily react with the photographic bath or take effect on the silver halide.

It has been found that diffusion of the dyestuffs in the layer may be prevented to a very considerable extent, if salts of the acid or substantive dyestuffs, and more particularly of the sulphonic acids of these dyestuffs, are introduced into the layer with nitrogenous organic bases. These substances also have no detrimental effect on the silver halide.

The salts in question may be incorporated in finished state in the layers or emulsions in fine suspension or by way of addition in a suitable

solvent, for example alcohol, or these deposits may be produced in the layer itself by double decomposition. These non-diffusing salts of the dyestuff may be incorporated in those layers, which consist of a plurality of part layers poured one over the other or of a plurality of particles such as result from the known re-emulsifying action of differently colored emulsions. They may also be formed by applying, atomizing or impressing the dyestuff on to a colloidal layer, whereby there is employed either a solution of the dyestuff salts, or the same may be employed together with the organic bases for coloring the arrangements as described, or the dyestuff deposit may be formed in the layer itself by way of double decomposition. This method of fixing dyestuffs may also be employed for other purposes, for example in the transfer method, in which, for example, an organic base is introduced into the colloid used for the transfer, and an insoluble non-diffusing salt of the dyestuff there formed after the transfer has taken place. In this method the transfer images are extremely sharp, owing to prevention of the diffusion. This method is also extremely useful for the production of anti-halo layers.

Layers containing, for example, substantive dyes, which may be removed entirely from the gelatine by washing, may be applied to the emulsion carrier on the front or the rear side of a film or plate or immediately above or below the emulsion.

For this purpose there is produced the suitable salt of an organic base, for example 2-phenyl-4-aminoquinoline, with Ponceau 4R. This salt may be split in a caustic alkaline developer and the dyestuff thereupon removed by washing.

The resulting salts possess varying powers of dissociation, and it is desirable for color photographic purposes to employ a merely weak alkaline neutral or acid developer.

## Examples

1. A 1% solution of Diamine pure blue FF (518) is admixed with a solution of guanidine sulphate. A deposit is formed, which is filtered.

2. Metanil yellow (138) is admixed with hydrochloric 2-phenyl-4-amino-quinoline.

The number of useful salt forming organic bases is extremely large. It is also possible to employ alkaloids, for instance quinine or cinchonine. The dyestuff is brought together with a salt of the bases in a solution and the resulting deposit subsequently dissolved in alcohol or another suitable solvent and added to the gelatine.

The procedure may also be such that the dyestuff is added to a part of the gelatine and one of the above salts to the rest of the gelatine. Or the layer may contain the bases and subsequently be colored with dyestuff, or, vice versa, the dyestuff may be included in the layer, and subsequently treated with a base for the purpose of producing the dyestuff deposit.

3. A colorless gelatine solution is admixed with 10 an alcoholic solution of hydrochloric 2-phenyl-4- amino-quinoline, and a fine grain suspension of the quinoline salt is caused. The gelatine is poured onto paper, and transfer images, for example pina type images, formed on the layers 15 thus produced. The resulting pictures are extremely sharp, owing to the lack of diffusion.

What I claim is:—

1. In a method of producing colored multi-layer photographic materials in which at least one colored emulsion is poured onto a support, the step which consists in coloring the emulsion by a water insoluble salt of an acid dyestuff and a 20

colorless nitrogenous organic base produced at a point in the process prior to coating by double decomposition of a water soluble salt of said colorless nitrogenous organic base and a water soluble salt of the said acid dyestuff.

2. In a method of producing colored multi-layer photographic materials in which at least one colored light-sensitive emulsion is poured onto a support, the step which consists in coloring the emulsion by a water insoluble salt of an 10 acid dyestuff and a colorless nitrogenous organic base produced in the emulsion at a point in the process prior to coating by double decomposition of a water soluble salt of said colorless nitrogenous organic base and a water soluble base of 15 the said acid dyestuff.

3. A photographic material consisting of a support and at least two superimposed layers, wherein at least one layer contains a substantially water insoluble salt of a colorless nitrogenous organic base and an acid dyestuff. 20

BÉLA GASPAR.